

July 3, 1956

G. P. HAMNER

2,753,326

## PETROLEUM RESINS FROM HEAVY FRACTIONS

Filed Jan. 8, 1953



Glen P. Hamner Inventor

By W. H. Smyers Attorney

## 1

2,753,326

## PETROLEUM RESINS FROM HEAVY FRACTIONS

Glen P. Hamner, Baton Rouge, La., assignor to Esso Research and Engineering Company, a corporation of Delaware

Application January 8, 1953, Serial No. 330,293

5 Claims. (Cl. 260—82)

This invention relates to the production of petroleum resins prepared from selected steam cracked distillate fractions and to the high softening point petroleum resins produced thereby.

Unsaturated petroleum fractions have been used as feeds for preparing hydrocarbon petroleum resins. For example, heavier petroleum fractions such as naphtha, gas oil, and the like, are cracked at relatively low pressure and at temperatures of 1000 to 1500° F. in the presence of steam and for relatively short contact times. The gas and liquid streams produced contain large quantities of diolefins and olefins in the C<sub>5</sub> to C<sub>10</sub> range. The naphtha distillate streams obtained by steam cracking operations contain large amounts of diolefins, olefins, aromatics and some paraffins.

The resins produced from these streams, however, have softening points that are generally too low for certain applications, such as, for example, in floor tile compositions. For use as the binding ingredient in floor tile, for example, it is desirable that hydrocarbon resins have softening points of about 95–100° C. or greater so that the floor tiles made therefrom have the required indentation characteristics, flexibility, and impact resistance. Most of the resins that are produced from such hydrocarbon streams by Friedel-Crafts polymerization have softening points lower than 100° C.

It has been discovered that naphtha streams produced from low pressure steam cracking of gas oil, naphtha, etc., contain large quantities of various diolefins (20–30 wt. per cent), olefins and aromatics. The diolefins may be recovered by thermal soaking in order to dimerize the active diolefins. It is necessary to prefractionate the naphtha. This is done in a manner wherein the lightest boiling diolefin monomers, when present as the dimers, will not boil in the boiling range of the heaviest diolefin monomers. After this thermal soaking, the dimers, codimers and trimers formed are recovered by distillation. In this distillation, the unreacted naphtha is taken as an overhead stream and the dimerized products are removed as a bottoms stream. The bottoms fraction thus obtained is then fed to a cracking zone whereby the material is heated to a temperature (400–700° F.) above the cyclodiolefin dimer cracking point. The total heated stream contains diolefins as the cyclic diolefin monomers and the non-cyclic diolefins as the dimer, codimer or higher homologs.

In order to carry out the invention, this total heated stream boiling from 80° to 580° F. from which polymeric and carbonaceous materials have previously been removed is preferably mixed with an inert solvent prior to polymerization. The stream boiling from 115° to 580° F. may also be employed. The preferred proportions are 2 parts solvent to 1 part of diolefins. Inert solvents such as aromatic or paraffin hydrocarbons can be used.

A steam cracked naphtha having a boiling range of 80 to 280° F. was thermally soaked at 300° F. for 6–8 hours. The pressure employed was the vapor pres-

## 2

sure of the liquid at this temperature; e. g., 100–400 p. s. i. g. A yield of 27.1 wt. per cent dimer or codimer was formed. The dimer product was removed from the naphtha by distillation. Analytical data obtained on this material are as follows:

VACUUM DISTILLATION, 30 PLATES, 10/1  
REFLUX RATIO

|                          | 10          | ° F. <sup>1</sup> | Refractive Index |
|--------------------------|-------------|-------------------|------------------|
| I. B. P.                 |             | 294               |                  |
| 5.                       | 337         | 1.4817            |                  |
| 10.                      | 339         | 1.4814            |                  |
| 20.                      | 352         | 1.4883            |                  |
| 15.                      | 363         | 1.4886            |                  |
| 30.                      | 376         | 1.4890            |                  |
| 40.                      | 390         | 1.4898            |                  |
| 50.                      | 395         | 1.4930            |                  |
| 60.                      | 430         | 1.4969            |                  |
| 70.                      | 470         | 1.5223            |                  |
| 80.                      | 570         |                   |                  |
| 90.                      | 710         | 1.5306            |                  |
| Btms.                    |             |                   |                  |
| Gravity, API @ 60° F.    |             | 21.7              |                  |
| Analysis by Ultraviolet: |             |                   |                  |
| Cyclopentadiene          | wt. percent | 26.6              |                  |
| Methylcyclopentadiene    | do          | 15.9              |                  |

<sup>1</sup> Temperature readings converted to atmospheric conditions.

After cracking at 400°–700° F., as above described, the mixture is subjected to a Friedel-Crafts catalyst such as BF<sub>3</sub>, AlCl<sub>3</sub>, or AlBr<sub>3</sub>, whereby the diolefin monomers and dimers are polymerized to a hard, resin product which remains substantially in solution in the inert diluent. The temperature of the polymerization may be between –20° and +200° F. The preferred limits are 0 to +100° F. The solvent plus the resin product and the excess catalyst is then contacted with alcohol and water to remove the catalyst. The water-washed mixture of solvent and resin is then fed to a fractionator to remove the solvent for recycling and the resin product is removed as a bottoms stream which may be subsequently stripped to any desired softening point.

If desired, other materials may be added to the polymerizing mixture in order to alter the properties of the product.

The invention will be described in greater detail by the following examples although it is not intended to limit the invention to the exact details disclosed therein.

*Example 1*

This invention can be more fully understood if the following example is read in conjunction with the accompanying schematic drawing.

Stream 1 containing C<sub>5</sub>, C<sub>6</sub>, and C<sub>7</sub> fraction (60–250° F.) obtained from steam cracking operations has about 20–25 wt. per cent diolefins, 30–35 wt. per cent aromatics, 2–4 wt. per cent paraffins and 35–40 wt. per cent olefins. These fractions are then thermally soaked in vessel A at 300–400° F. and 100–400 pounds pressure for 8–10 hours. The thermally soaked naphtha stream 2 which is produced contains approximately 20 wt. per cent diolefin dimers and the other components above. To recover the dimers, stream 2 is fed to tower B, taking overhead stream 3 and part of this condensate is returned through line 4 as reflux. Stream 3 contains C<sub>5</sub>, C<sub>6</sub> and C<sub>7</sub> fractions which are relatively free of diolefins. The dimer product (C<sub>10</sub>–C<sub>14</sub>) is removed as a bottoms stream 5. Part of this stream is returned to tower B through line 6 to furnish heat to the tower. Stream 7 is then C<sub>10</sub>–C<sub>14</sub> components (C<sub>5</sub>, C<sub>6</sub>, C<sub>7</sub> diolefin dimers or codimers) and any recycle streams 22 which are fed to cracking zone C. The cracking zone C is maintained at 350–900° F., preferably 400–700° F., and 0–10 pounds pressure. Stream 8 from the crack-

ing zone then contains 50-60% monomers of cyclopentadiene, methylcyclopentadiene, dimethylcyclopentadiene, and other cyclic diolefins and 40-50% uncracked dimers or codimers of isoprene, piperylene, hexadienes, heptadienes and other non-cyclic diolefins. This mixture of diolefin monomers and dimers is fed to tower D. An overhead vapor of C<sub>8</sub> components (68-110° F.) is removed overhead as stream 9 and part of the condensed stream recycled through line 10 to the top tray as reflux. The overhead product (stream 9) is 90-95 wt. per cent cyclopentadiene. The tower is operated with the minimum reflux ratio (1/1) required to produce a greater than 90% cyclopentadiene overhead stream. It may be desirable to operate under reduced pressures to minimize any dimerization of cyclopentadienes back to the dimer without the tower. A mixture of methylcyclopentadiene, dimethylcyclopentadiene, and other cyclic diolefin monomers together with the uncracked dimers are removed from the tower as bottoms stream 11. Part of this stream may be recycled to the cracker by line 22. A part of stream 11 is returned to tower D by line 21 to furnish heat to the tower. The remainder of the stream is combined with a diluent (C<sub>6</sub>-C<sub>7</sub> paraffins or aromatics) to form the polymerization feed stream. The solvent is added by line 14 to keep the resin formed in solution. Catalyst is added by line 13. The polymerization is conducted in reactor E with BF<sub>3</sub> or AlCl<sub>3</sub> catalyst. Polymerization conditions are 10-60 minutes at 0 to 100° F. for BF<sub>3</sub> catalyst <200° F. for AlCl<sub>3</sub> catalyst. The polymerized material in solution with the solvent is passed from the reactor by line 23 and is water-washed in vessel F. Steam may be added by line 17. Water or steam condensate with the catalyst is removed through line 16. The solvent and the resin product are removed through line 15 and fed to the second tray of tower G. Stream 24 is the solvent and unreacted portion which are taken overhead to be recycled back to the polymerization reactor E fed by line 12. Part of stream 24 is recycled through line 19 as reflux to the first tray from the top of tower G. The polymerized product is removed as a bottoms stream 18 and may be subjected to further treatment and purification, if desired.

## Example 2

A sample of uncracked dimers was blended with the methylcyclopentadiene - dimethylcyclopentadiene monomer from the same product. Xylene solvent was used to dilute the above blend before polymerization with excess BF<sub>3</sub> gas at 40-80° F. for 20-30 minutes. A yield of >95% resin based on non-aromatic components, having a softening point of 280° F., and an iodine number of >400, was obtained. Normally, resins having softening point of <200° F. and iodine numbers of 300 are obtained when polymerizing such components in the presence of the original unprocessed feed to the thermal soaker A or when treating stream 5 (dimers of the various diolefins) as polymerization feed.

The unprocessed 60-250° F. feed to the thermal soaker A was polymerized with excess BF<sub>3</sub> gas at 30-40° F. for 30 minutes. A yield of 39.9 wt. per cent polymeric resin was obtained having the following properties.

Softening point, ° F. ..... <120  
Iodine number (cg./g.) ..... 239  
Color<sup>1</sup> ..... 1  
Gravity, API @ 60° F. ..... 15.9

<sup>1</sup> 1 gr. polymeric resin in 67 ml. xylene.

The naphtha feed was thermally soaked at 220° F. for 8-10 hours prior to polymerization. The naphtha containing all the dimerized diolefins (mostly cyclic (70-80%) since only thermally soaked, at 220° F.) was polymerized with excess BF<sub>3</sub> at 30-40° F. for 30 minutes.

A yield of 34.3 wt. per cent polymeric resin was obtained having the following properties.

5 Softening pt., ° F. ..... <120  
Iodine number (cg./g.) ..... 242  
Color<sup>1</sup> ..... 1  
Gravity ..... 14.9

<sup>1</sup> 1 gr. polymeric resin in 67 ml. xylene.

In each of the above two examples a polymeric resin product was obtained when polymerizing the cracked naphtha containing diolefins as monomers and dimers. A higher yield was obtained when most of the diolefin components were present as the monomer. The resin produced by BF<sub>3</sub> polymerizing diolefin monomers and dimers in an inert solvent has a higher softening point and is considerably more unsaturated.

When AlCl<sub>3</sub> polymerizing the unprocessed feed to thermal soaker A at 40 to 80° F. for 30 minutes a yield of 30 to 35 wt. per cent resin is obtained. Inspection on this resin is as follows.

20 Softening pt., ° F. ..... 185 to 200  
Iodine number ..... 170 to 200  
Color ..... 2 to 3

25 These data show that a resin of lower softening point and unsaturation is formed when AlCl<sub>3</sub> polymerizing the diolefins in the presence of the cracked naphthas (olefins).

## Example 3

30 A sample of dimer concentrates (as stream 7) was cracked and cyclopentadiene removed from the cracked products by fractionation (stream 9). The bottoms containing about 24 weight per cent cyclopentadiene and 53.7 weight per cent methylcyclopentadiene, along with other cyclic and acyclic diolefins, was then polymerized at 35-40° C. using various quantities of AlCl<sub>3</sub> as the catalyst. The reaction products were washed to remove residual catalyst and then stripped to a resin (bottoms) temperature of 260° C. at 5 mm. Hg. Data relating to these polymerizations follow:

| Wt. Per-<br>cent<br>AlCl <sub>3</sub> | Wt. Per-<br>cent<br>Resin | Resin Properties |       |                  |
|---------------------------------------|---------------------------|------------------|-------|------------------|
|                                       |                           | Soft<br>Pt., °F. | Color | Iodine<br>Number |
| 0.7.....                              | 20.5                      | 283              | 9     | 267              |
| 1.0.....                              | 39.7                      | 320              | 7     | 246              |

50 55 60 65 70 75 80 85 90 95 100

What is claimed is:

1. An improved process for preparing petroleum hydrocarbon resins which comprises subjecting a cracked naphtha stream boiling from 80 to 280° F. to thermal soaking to dimerize the cyclic and non-cyclic diolefins, separating and heating the dimerized product at 400 to 700° F. whereby the cyclic diolefin dimers are cracked to monomers and the non-cyclic diolefin dimers remain uncracked, and polymerizing the resulting stream with a boron fluoride catalyst at a temperature in the range between 0 and 200° F. for a time between 10 and 30 minutes and isolating the resin produced thereby.
2. An improved process for preparing a petroleum resin which comprises subjecting a naphtha comprising cyclic diolefins, acyclic diolefins, mono-olefins, aromatics and paraffins which has been cracked at about 1000°-1500° F. to dimerization, separating a fraction in which the polymerizable materials consist of the dimers of acyclic and cyclic diolefins, heating said dimers at a temperature sufficient to crack the cyclic diolefin dimers to monomers, the acyclic diolefin dimers remaining uncracked, polymerizing the resulting stream with a Friedel-Crafts catalyst to produce a hydrocarbon resin, and recovering the resin produced thereby.
3. A petroleum resin having a softening point of at

least about 280° F. and an iodine number above about 400 cg./g. produced by the process of claim 2.

4. Process according to claim 2 in which cyclopentadiene is removed prior to polymerization.

5. A petroleum hydrocarbon resin having a softening point of at least about 280° F. and an iodine number above about 400 cg./g. which has been produced by the process of claim 4.

## References Cited in the file of this patent

## UNITED STATES PATENTS

|           |         |               |
|-----------|---------|---------------|
| 1,836,629 | Thomas  | Dec. 15, 1931 |
| 1,982,708 | Thomas  | Dec. 4, 1934  |
| 2,255,409 | Carmody | Sept. 9, 1941 |
| 2,352,980 | Soday   | July 4, 1944  |
| 2,521,022 | Rowland | Sept. 5, 1950 |
| 2,608,550 | Rowland | Aug. 26, 1952 |